

## [54] VOLTAGE-NONLINEAR RESISTORS

[75] Inventors: **Mikio Matsuura; Atsushi Iga; Yasuo Wakahata**, all of Osaka, Japan

[73] Assignee: **Matsushita Electric Industrial Co., Ltd.**, Osaka, Japan

[22] Filed: **Aug. 14, 1973**

[21] Appl. No.: **388,169**

## [30] Foreign Application Priority Data

Aug. 14, 1972 Japan ..... 47-81643

[52] U.S. Cl. .... **338/20**, 252/518, 338/21

[51] Int. Cl. .... **H01c 7/10**

[58] Field of Search ..... 338/20, 21; 252/518-520

## [56] References Cited

## FOREIGN PATENTS OR APPLICATIONS

831,691 1/1970 Canada ..... 338/20

Primary Examiner—C. L. Albritton

Attorney, Agent, or Firm—Wenderoth, Lind & Ponack

## [57] ABSTRACT

The invention relates to voltage-nonlinear resistors having nonohmic resistance due to the bulk thereof and more particularly to varistors, which utility as surge absorbers and D.C. stabilizers, comprising zinc oxide, bismuth oxide, cobalt oxide, boron trioxide and at least one member selected from the group consisting of magnesium oxide, calcium oxide, barium oxide and strontium oxide.

5 Claims, 1 Drawing Figure



Patented Jan. 28, 1975

3,863,193



**VOLTAGE-NONLINEAR RESISTORS**

Various voltage-nonlinear resistors such as silicon carbide varistors, selenium rectifiers and germanium or silicon p-n junction diodes have been widely used for stabilization of voltage of electrical circuits or suppression of abnormally high surge induced in electrical circuits. The electrical characteristics of such nonlinear resistors are expressed by the relation:

$$I = (V/C)^n \quad (1)$$

where  $V$  is the voltage across the resistor,  $I$  is the current flowing through the resistor,  $C$  is a constant corresponding to the voltage at a given current and exponent  $n$  is a numerical value greater than 1. The value of  $n$  is calculated by the following equation:

$$n = \log_{10}(I_2/I_1)/\log_{10}(V_2/V_1) \quad (2)$$

where  $V_1$  and  $V_2$  are the voltages at given currents  $I_1$  and  $I_2$ , respectively. The desired value of  $C$  depends upon the kind of application to which the resistor is to be put. It is ordinarily desirable that the value of  $n$  be as large as possible since this exponent determines the extent to which the resistors depart from ohmic characteristics.

Nonlinear resistors comprising sintered bodies of zinc oxide with or without additives and non-ohmic electrode applied thereto, have already been disclosed as seen in U.S. Pat. Nos. 3,496,512, 3,570,002, 3,503,029 and 3,689,863. The nonlinearity of such varistors is attributed to the interface between the sintered body of zinc oxide with or without additives and silver paint electrode, and is controlled mainly by changing the compositions of said sintered body and silver paint electrode. Therefore, it is not easy to control the  $C$ -value over a wide range after the sintered body is prepared. Similarly, in varistors comprising germanium or silicon p-n junction diodes, it is difficult to control the  $C$ -value over a wide range because the nonlinearity of these varistors is not attributed to the bulk but rather to the p-n junction. In addition, it is almost impossible for those zinc oxide varistors mentioned above and germanium or silicon diode varistors to obtain the combination of  $C$ -value higher than 100 volt,  $n$ -value higher than 10 and high surge resistance tolerable for surge more than 100Ap.

On the other hand, the silicon carbide varistors have nonlinearity due to the contacts among the individual grains of silicon carbide bonded together by a ceramic binding material, i.e. to the bulk, and  $C$ -value is controlled by changing a dimension in the direction in which the current flows through the varistors. In addition, the silicon carbide varistors have high surge resistance thus rendering them suitable as surge absorbers. The silicon carbide varistors, however, have a relatively low  $n$ -value ranging from 3 to 7 which results in poor surge suppression as well as poor D.C. stabilization. Another defect of the silicon carbide varistor as a D.C. stabilizer is their change in  $C$ -value and  $n$ -value during D.C. load application.

There have been known, on the other hand, voltage-nonlinear resistors of bulk type comprising a sintered body of zinc oxide with additives, as seen in U.S. Pat. Nos. 3,663,458, 3,632,529, 3,634,337, 3,598,763,

3,682,841, 3,642,664, 3,658,725 and 3,687,871, and U.S. Patent copending application No. 29,416. These zinc oxide varistors contain, as additives, one or more combinations of oxides or fluorides of bismuth, cobalt, manganese, barium, boron, magnesium, calcium, strontium, titanium, antimony chromium and nickel, and are controllable in  $C$ -value by changing the distance between electrodes and have an excellent nonlinear property in an  $n$ -value. The power dissipation for surge energy, however, shows a relatively low value compared with that of the conventional silicon carbide varistor, so that the change rate of  $C$ -value exceeds 20 percent after two standard surges of  $8 \times 20 \mu\text{sec}$  wave form in a peak current of  $500\text{A}/\text{cm}^2$  are applied to said zinc oxide varistors of bulk type. Another defect of these zinc oxide varistors of bulk type is in their poor stability for D.C. load, particularly in their remarkable decreases of  $C$ -value measured in a low current region such as  $0.1\text{mA}$  and  $0.01\text{mA}$  after applying high D.C. power. This deterioration in the  $C$ -value is unfavorable for a voltage stabilizer which devices require high accuracy and low loss.

An object of the present invention is to provide a voltage-nonlinear resistor having high  $n$ -value, high power dissipation for surge energy and high stability for D.C. load even in a range of current less than  $0.1\text{mA}/\text{cm}^2$ .

This object of the invention will become apparent upon consideration of the following description taken together with the accompanying drawing in which the FIGURE is a cross-sectional view through a voltage-nonlinear resistor in accordance with the invention.

Before proceeding with a detailed description of the voltage-nonlinear resistor contemplated by the invention, its construction will be described with reference to the aforesaid figure of drawing wherein reference character 10 designates, as a whole, a voltage-nonlinear resistor comprising, as its active element, a sintered body having a pair of electrodes 2 and 3 in an ohmic contact applied to opposite surfaces thereof. Said sintered body 1 is prepared in a manner hereinafter set forth and is any form such as circular, square or rectangular plate form. Wire leads 5 and 6 are attached conductively to the electrodes 2 and 3, respectively, by a connection means 4 such as solder or the like.

A voltage-nonlinear resistor according to the invention comprises a sintered body of a composition comprising, as an additive, 0.01 to 10.0 mole percent of bismuth oxide ( $\text{Bi}_2\text{O}_3$ ), 0.01 to 10 mole percent of cobalt oxide ( $\text{Co}_2\text{O}_3$ ), 0.01 to 5.0 mole percent of boron trioxide ( $\text{B}_2\text{O}_3$ ) and 0.01 to 5.0 mole percent of at least one member selected from the group consisting of magnesium oxide ( $\text{MgO}$ ), calcium oxide ( $\text{CaO}$ ), barium oxide ( $\text{BaO}$ ), strontium oxide ( $\text{SrO}$ ) and the remainder of zinc oxide ( $\text{ZnO}$ ) as a main constituent, and electrodes applied to opposite surfaces of said sintered body. Such a voltage-nonlinear resistor has non-ohmic resistance due to the bulk itself. Therefore, its  $C$ -value can be changed without impairing the  $n$ -value by changing the distance between said opposite surfaces. According to the invention, said resistor has high  $n$ -value and high stability for D.C. load.

The higher stability with respect to D.C. load and surge pulses can be obtained when said additive consists essentially of 0.1 to 3.0 mole percent of bismuth oxide ( $\text{Bi}_2\text{O}_3$ ), 0.1 to 3.0 mole percent of cobalt oxide ( $\text{Co}_2\text{O}_3$ ), 0.01 to 5.0 mole percent of boron trioxide

( $B_2O_3$ ) and 0.01 to 5.0 mole percent of at least one member selected from the group consisting of magnesium oxide ( $MgO$ ), calcium oxide ( $CaO$ ), barium oxide ( $BaO$ ) and strontium oxide ( $SrO$ ).

It has been discovered according to the present invention that the higher  $n$ -value and higher stability with respect to D.C. load and surge power can be obtained when said additive consists essentially of 0.1 to 3.0 mole percent of bismuth oxide ( $Bi_2O_3$ ), 0.1 to 3.0 mole percent of cobalt oxide ( $Co_2O_3$ ), 0.01 to 5.0 mole percent of boron trioxide ( $B_2O_3$ ), 0.01 to 5.0 mole percent of at least one member selected from the group consisting of magnesium oxide ( $MgO$ ), calcium oxide ( $CaO$ ), barium oxide ( $BaO$ ) and strontium oxide ( $SrO$ ), and 0.1 to 3.0 mole percent of manganese oxide ( $MnO$ ).

According to the present invention, the  $n$ -value and stability with D.C. load and surge power can be further improved and the C-value can be controlled when said additive consists essentially of 0.1 to 3.0 mole percent of bismuth oxide ( $Bi_2O_3$ ), 0.1 to 3.0 mole percent of cobalt oxide ( $Co_2O_3$ ), 0.01 to 5.0 mole percent of boron trioxide ( $B_2O_3$ ) and 0.01 to 5.0 mole percent of at least one member selected from the group consisting of magnesium oxide ( $MgO$ ), calcium oxide ( $CaO$ ), barium oxide ( $BaO$ ) and strontium oxide ( $SrO$ ), 0.1 to 3.0 mole percent of manganese oxide ( $MnO$ ) and one member selected from the group consisting of 0.05 to 3.0 mole percent of antimony oxide ( $Sb_2O_3$ ) and 0.1 to 3.0 mole percent of titanium oxide ( $TiO_2$ ). The addition of antimony oxide increases the C-value of the resultant voltage-nonlinear resistor and the addition of titanium oxide lowers the C-value of the resultant voltage nonlinear resistor.

According to the present invention, the stability with D.C. load and the stability for surge pulses can be remarkably improved when said sintered body comprises, as a main constituent, zinc oxide ( $ZnO$ ) and, as an additive, 0.1 to 3.0 mole percent of bismuth oxide ( $Bi_2O_3$ ), 0.1 to 3.0 mole percent of cobalt oxide ( $Co_2O_3$ ), 0.1 to 3.0 mole percent of manganese oxide ( $MnO$ ), 0.01 to 5.0 mole percent of boron trioxide ( $B_2O_3$ ), 0.1 to 3.0 mole percent of titanium oxide ( $TiO_2$ ), at least one member selected from the group consisting of 0.01 to 3.0 mole percent of chromium oxide ( $Cr_2O_3$ ) and 0.1 to 3.0 mole percent of nickel oxide ( $NiO$ ), and 0.01 to 5.0 mole percent of at least one member selected from the group consisting of magnesium oxide ( $MgO$ ), calcium oxide ( $CaO$ ), barium oxide ( $BaO$ ) and strontium oxide ( $SrO$ ).

The sintered body I can be prepared by a per se well known ceramic technique. The starting materials in the compositions in the foregoing description are mixed in a wet mill so as to produce homogeneous mixtures. The mixtures are dried and pressed in a mold into desired shapes at a pressure from 50  $Kg./cm^2$  to 500  $Kg./cm^2$ . The pressed bodies are sintered in air at 1,000° to 1,450°C for 1 to 20 hours, and then furnace-cooled to room temperature (about 15°C to about 30°C). The mixtures can be preliminarily calcined at 700° to 1,000°C and pulverized for easy fabrication in the subsequent pressing step. The mixture to be pressed can be admixed with a suitable binder such as water, polyvinyl alcohol, etc. It is advantageous that the sintered body be lapped at the opposite surfaces by abrasive powder such as silicon carbide in a particle size of 50  $\mu$  in mean diameter to 10  $\mu$  in mean diameter. The sintered bodies are provided, at the opposite surfaces thereof with elec-

trodes in any available and suitable method such as silver painting, vacuum evaporation or flame spraying of metal such as Al, Zn, Sn etc.

The voltage-nonlinear properties are not practically affected by the kind of electrodes used, but are affected by the thickness of the sintered bodies. Particularly, the C-value varies in proportion to the thickness of the sintered bodies, while the  $n$ -value is almost independent of the thickness. This surely means that the voltage-nonlinear property is due to the bulk itself, but not to the electrodes.

Lead wires can be attached to the electrodes in a per se conventional manner by using conventional solder. It is convenient to employ a conductive adhesive comprising silver powder and resin in an organic solvent in order to connect the lead wires to the electrodes. Voltage-nonlinear resistors according to this invention have a high stability to temperature, for the D.C. load test, which is carried out by applying a rating power of 1 watt at 70°C ambient temperature for 500 hours, and for the surge test, which is carried out by applying surge wave form of  $8 \times 20 \mu$ sec, 500A/cm<sup>2</sup>. The  $n$ -value do not change remarkably after the heating cycles, the load life test, humidity test, and surge test. Particularly, the C-value and  $n$ -value do not change so much even in a region of the current less than 0.1mA after DC. load life test. It is advantageous for achievement of a high stability with respect to humidity that the resultant voltage-nonlinear resistors be embedded in a humidity proof resin such as epoxy resin and phenol resin in a per se well known manner. Presently preferred illustrative embodiments of the invention are as follows.

#### EXAMPLE 1

35 Starting material composed of 97.0 mole percent of zinc oxide, 1.0 mole percent of bismuth oxide, 1.0 mole percent of cobalt oxide, and 0.5 mole percent of boron trioxide and 0.5 mole percent of magnesium oxide is mixed in a wet mill for 24 hours. The mixture is dried and pressed in a mold into discs of 17.5mm in diameter and 7mm in thickness at a pressure of 250  $Kg./cm^2$ .

40 The pressed bodies are sintered in air at the condition shown in Table 1, and then furnace-cooled to room temperature. The sintered body is lapped at the opposite surfaces thereof into the thickness shown in Table 1 by silicon carbide abrasive in particle size of 30  $\mu$  in mean diameter. The opposite surfaces of the sintered body are provided with a spray metallized film of aluminum in a per se well known technique.

45 50 The electric characteristics of resultant sintered body are shown in Table 1, which shows that the C-value varies approximately in proportion to the thickness of the sintered body while the  $n$ -value is essentially independent of the thickness. It will be readily realized that the voltage-nonlinear property of the sintered body is attributed to the sintered body itself.

#### EXAMPLE 2

55 60 Zinc oxide and with additives listed in Table 2 are fabricated into voltage-nonlinear resistors by the same process as that of Example 1. The thickness is 1.0 mm. The resulting electrical properties are shown in Table 2, in which the value of  $n$  are the  $n$ -values defined between 0.1mA and 1mA. The test is carried out by applying D.C. load of 1 watt at 70°C ambient temperature for 500 hours. It can be easily understood that the combined addition of bismuth oxide, cobalt oxide, boron

trioxide and one member selected from the group consisting of magnesium oxide, calcium oxide, barium oxide and strontium oxide, as additives shows the high  $n$ -value and small change rates.

#### EXAMPLE 3

Zinc oxide and additives of Table 3 are fabricated into the voltage-nonlinear resistors by the same process as that of Example 2. The electrical properties of the resultant resistors are shown in Table 3. The change rates of  $C$  and  $n$  values after D.C. load and impulse test are also shown in Table 3. The impulse test is carried out by applying two impulses of  $8 \times 20 \mu\text{sec}$ , 500A, and D.C. load life test is carried out by the same method as that of Example 2. It will be readily realized that the further addition of manganese oxide results in the higher  $n$ -value and smaller change rates than those of Example 2.

#### EXAMPLE 4

Zinc oxide and additives of Table 4 are fabricated into the voltage-nonlinear resistors by the same process as Example 2. The electrical characteristics of resulting resistors are shown in Table 4. It will be easily understood that the further addition of one member selected from the group consisting of antimony oxide and titanium oxide results in the higher  $n$ -value and smaller change rates than those of Example 3. The change rates of  $C$  and  $n$  values after D.C. and impulse test carried out by the same method as that of Example 3 are also shown in Table 4.

#### EXAMPLE 5

Zinc oxide and additives of Table 5 are fabricated into the voltage-nonlinear resistors by the same process as Example 2. The electrical characteristics of resultant resistors are shown in Table 5. It will be easily understood that the further addition of nickel oxide and chromium oxide results in the higher  $n$ -value and smaller change rates than those of Example 4. The change rates of  $C$  and  $n$  values after D.C. test and im-

pulse test carried out by the same method as those of Example 3 are also shown in Table 5.

#### EXAMPLE 6

The resistors of Example 2,3,4 and 5 are tested in accordance with a method widely used in the electronic component parts. The heating cycle test is carried out by repeating five times the cycle in which said resistors are kept at  $85^\circ\text{C}$  ambient temperature for 30 minutes, cooled rapidly to  $-20^\circ\text{C}$  and then kept at such temperature for 30 minutes. The humidity test is carried out at  $40^\circ\text{C}$  and 95 percent relative humidity for 1,000 hrs. Table 6 shows the average change rates of  $C$ -value and  $n$ -value of resistors after heating cycle test and humidity test. It is easily understood that each sample has a small change rate.

Table 6

| Sample No. | Heating Cycle Test (%) |      | Humidity Test (%) |      |
|------------|------------------------|------|-------------------|------|
|            | $c$                    | $n$  | $c$               | $n$  |
| Example 2  | -4.9                   | -6.5 | -5.2              | -6.8 |
| Example 3  | -2.8                   | -5.7 | -3.7              | -5.4 |
| Example 4  | -1.8                   | -3.9 | -1.1              | -3.7 |
| Example 5  | -1.0                   | -2.5 | -0.8              | -2.2 |

Table 1

| Thickness (mm) | $c$<br>(at 1mA) | $n$ | Sintering Condition |                                 |
|----------------|-----------------|-----|---------------------|---------------------------------|
|                |                 |     | initial             | do.                             |
| initial        | (5)             | 680 | 24                  | $1200^\circ\text{C}$ , 5 Hours  |
|                | 2               | 275 | 24                  | do.                             |
|                | 1               | 135 | 23                  | do.                             |
|                | 0.5             | 68  | 23                  | do.                             |
| initial        | (5)             | 600 | 24                  | $1350^\circ\text{C}$ , 1 Hour   |
|                | 2               | 240 | 24                  | do.                             |
|                | 1               | 120 | 23                  | do.                             |
|                | 0.5             | 60  | 23                  | do.                             |
| initial        | (5)             | 850 | 23                  | $1000^\circ\text{C}$ , 20 Hours |
|                | 2               | 330 | 23                  | do.                             |
|                | 1               | 170 | 23                  | do.                             |
|                | 0.5             | 85  | 23                  | do.                             |

Table 2

| $\text{Bi}_2\text{O}_3$ | $\text{Co}_2\text{O}_3$ | $\text{B}_2\text{O}_3$ | $\text{MgO}$ | Additives (mole %) |     | Electrical Properties of Resultant Resistor |      | Change Rate after Test (%) |      |
|-------------------------|-------------------------|------------------------|--------------|--------------------|-----|---------------------------------------------|------|----------------------------|------|
|                         |                         |                        |              | $c$<br>at 1 mA     | $n$ | $c$<br>at 0.01 mA                           | $n$  | $c$<br>at 0.01 mA          | $n$  |
| 0.01                    | 3.0                     | 0.5                    | 0.5          | 57                 | 20  | -4.3                                        | -4.3 | -2.6                       | -2.1 |
| 0.1                     | 3.0                     | 0.5                    | 0.5          | 79                 | 20  | -2.6                                        | -2.3 | -2.4                       | -2.3 |
| 1.0                     | 3.0                     | 0.5                    | 0.5          | 133                | 23  | -2.4                                        | -2.4 | -2.5                       | -2.4 |
| 3.0                     | 3.0                     | 0.5                    | 0.5          | 141                | 22  | -4.9                                        | -4.4 | -4.5                       | -4.4 |
| 10.0                    | 3.0                     | 0.5                    | 0.5          | 149                | 22  | -4.8                                        | -4.8 | -2.4                       | -2.2 |
| 3.0                     | 0.01                    | 0.5                    | 0.5          | 69                 | 18  | -2.4                                        | -2.4 | -2.3                       | -2.3 |
| 3.0                     | 0.1                     | 0.5                    | 0.5          | 125                | 20  | -2.1                                        | -2.1 | -2.6                       | -2.6 |
| 3.0                     | 1.0                     | 0.5                    | 0.5          | 129                | 22  | -2.7                                        | -2.7 | -2.3                       | -2.3 |
| 3.0                     | 3.0                     | 0.5                    | 0.5          | 137                | 20  | -2.7                                        | -2.7 | -2.6                       | -2.6 |
| 3.0                     | 10.0                    | 0.5                    | 0.5          | 158                | 19  | -4.9                                        | -4.9 | -5.0                       | -5.0 |
| 3.0                     | 3.0                     | 0.01                   | 0.5          | 117                | 25  | -2.9                                        | -2.9 | -2.5                       | -2.5 |
| 3.0                     | 3.0                     | 0.1                    | 6.5          | 125                | 23  | -2.7                                        | -2.7 | -2.4                       | -2.4 |
| 3.0                     | 3.0                     | 1.0                    | 0.5          | 123                | 26  | -2.3                                        | -2.3 | -2.4                       | -2.4 |
| 3.0                     | 3.0                     | 5.0                    | 0.5          | 142                | 27  | -2.6                                        | -2.6 | -2.5                       | -2.5 |
| 3.0                     | 3.0                     | 0.5                    | 0.01         | 137                | 25  | -2.8                                        | -2.8 | -2.2                       | -2.2 |
| 3.0                     | 3.0                     | 0.5                    | 0.1          | 126                | 23  | -2.7                                        | -2.7 | -2.2                       | -2.2 |
| 3.0                     | 3.0                     | 0.5                    | 1.0          | 122                | 23  | -2.6                                        | -2.6 | -2.4                       | -2.4 |
| 3.0                     | 3.0                     | 0.5                    | 5.0          | 106                | 25  | -2.7                                        | -2.7 | -2.4                       | -2.4 |
| $\text{Bi}_2\text{O}_3$ | $\text{Co}_2\text{O}_3$ | $\text{B}_2\text{O}_3$ | $\text{CaO}$ |                    |     |                                             |      |                            |      |
| 0.01                    | 3.0                     | 0.5                    | 0.5          | 58                 | 19  | -4.2                                        | -4.2 | -2.5                       | -2.2 |
| 0.1                     | 3.0                     | 0.5                    | 0.5          | 78                 | 21  | -2.5                                        | -2.3 | -2.2                       | -2.2 |
| 1.0                     | 3.0                     | 0.5                    | 0.5          | 134                | 22  | -2.4                                        | -2.4 | -2.5                       | -2.5 |
| 3.0                     | 3.0                     | 0.5                    | 0.5          | 142                | 22  | -4.1                                        | -4.1 | -4.5                       | -4.5 |
| 10.0                    | 3.0                     | 0.5                    | 0.5          | 148                | 23  | -4.7                                        | -4.7 | -4.4                       | -4.4 |
| 3.0                     | 0.01                    | 0.5                    | 0.5          | 70                 | 17  |                                             |      |                            |      |

Table 2 - Continued

| Additives (mole %)             |                                |                               |      | Electrical Properties of Resultant Resistor |                   | Change Rate after Test (%) |                   |
|--------------------------------|--------------------------------|-------------------------------|------|---------------------------------------------|-------------------|----------------------------|-------------------|
| Bi <sub>2</sub> O <sub>3</sub> | Co <sub>2</sub> O <sub>3</sub> | B <sub>2</sub> O <sub>3</sub> | MgO  | <sup>c</sup><br>at 1 mA                     | <sup>c</sup><br>n | <sup>c</sup><br>at 0.01 mA | <sup>c</sup><br>n |
| 3.0                            | 0.1                            | 0.5                           | 0.5  | 124                                         | 21                | -2.3                       | -2.3              |
| 3.0                            | 1.0                            | 0.5                           | 0.5  | 130                                         | 21                | -2.0                       | -2.2              |
| 3.0                            | 3.0                            | 0.5                           | 0.5  | 140                                         | 20                | -2.5                       | -2.4              |
| 3.0                            | 10.0                           | 0.5                           | 0.5  | 157                                         | 20                | -3.8                       | -4.1              |
| 3.0                            | 3.0                            | 0.01                          | 0.5  | 118                                         | 24                | -2.9                       | -2.4              |
| 3.0                            | 3.0                            | 0.1                           | 0.5  | 124                                         | 24                | -2.6                       | -2.5              |
| 3.0                            | 3.0                            | 1.0                           | 0.5  | 124                                         | 25                | -2.2                       | -2.3              |
| 3.0                            | 3.0                            | 5.0                           | 0.5  | 141                                         | 28                | -2.5                       | -2.6              |
| 3.0                            | 3.0                            | 0.5                           | 0.01 | 138                                         | 24                | -2.9                       | -2.8              |
| 3.0                            | 3.0                            | 0.5                           | 0.1  | 125                                         | 24                | -2.6                       | -2.3              |
| 3.0                            | 3.0                            | 0.5                           | 1.0  | 123                                         | 22                | -2.5                       | -2.3              |
| 3.0                            | 3.0                            | 0.5                           | 5.0  | 105                                         | 26                | -2.6                       | -2.5              |
| Bi <sub>2</sub> O <sub>3</sub> | Co <sub>2</sub> O <sub>3</sub> | B <sub>2</sub> O <sub>3</sub> | BaO  |                                             |                   |                            |                   |
| 0.01                           | 3.0                            | 0.5                           | 0.5  | 56                                          | 18                | -4.8                       | -4.5              |
| 0.1                            | 3.0                            | 0.5                           | 0.5  | 77                                          | 19                | -2.5                       | -2.4              |
| 1.0                            | 3.0                            | 0.5                           | 0.5  | 132                                         | 21                | -2.3                       | -2.5              |
| 3.0                            | 3.0                            | 0.5                           | 0.5  | 141                                         | 21                | -2.7                       | -2.9              |
| 10.0                           | 3.0                            | 0.5                           | 0.5  | 147                                         | 21                | -4.0                       | -4.7              |
| 3.0                            | 0.01                           | 0.5                           | 0.5  | 68                                          | 16                | -4.0                       | -4.2              |
| 3.0                            | 0.1                            | 0.5                           | 0.5  | 123                                         | 19                | -2.5                       | -2.5              |
| 3.0                            | 1.0                            | 0.5                           | 0.5  | 128                                         | 20                | -2.4                       | -2.5              |
| 3.0                            | 3.0                            | 0.5                           | 0.5  | 139                                         | 20                | -2.7                       | -2.9              |
| 3.0                            | 10.0                           | 0.5                           | 0.5  | 156                                         | 18                | -4.6                       | -4.3              |
| 3.0                            | 3.0                            | 0.01                          | 0.5  | 116                                         | 23                | -2.9                       | -2.9              |
| 3.0                            | 3.0                            | 0.1                           | 0.5  | 123                                         | 22                | -2.5                       | -2.7              |
| 3.0                            | 3.0                            | 1.0                           | 0.5  | 122                                         | 24                | -2.1                       | -2.6              |
| 3.0                            | 3.0                            | 5.0                           | 0.5  | 140                                         | 26                | -2.0                       | -2.8              |
| 3.0                            | 3.0                            | 3.0                           | 0.01 | 136                                         | 23                | -2.8                       | -2.8              |
| 3.0                            | 3.0                            | 3.0                           | 0.1  | 124                                         | 22                | -2.4                       | -2.5              |
| 3.0                            | 3.0                            | 3.0                           | 1.0  | 121                                         | 21                | -2.0                       | -2.6              |
| 3.0                            | 3.0                            | 3.0                           | 5.0  | 104                                         | 24                | -2.2                       | -2.7              |
| Bi <sub>2</sub> O <sub>3</sub> | Co <sub>2</sub> O <sub>3</sub> | B <sub>2</sub> O <sub>3</sub> | SrO  |                                             |                   |                            |                   |
| 0.01                           | 3.0                            | 0.5                           | 0.5  | 57                                          | 19                | -4.3                       | -4.5              |
| 0.1                            | 3.0                            | 0.5                           | 0.5  | 77                                          | 19                | -2.4                       | -2.3              |
| 1.0                            | 3.0                            | 0.5                           | 0.5  | 133                                         | 22                | -2.4                       | -2.3              |
| 3.0                            | 3.0                            | 0.5                           | 0.5  | 139                                         | 21                | -2.5                       | -2.9              |
| 10.0                           | 3.0                            | 0.5                           | 0.5  | 147                                         | 21                | -4.7                       | -4.0              |
| 3.0                            | 0.01                           | 0.5                           | 0.5  | 69                                          | 17                | -4.8                       | -4.8              |
| 3.0                            | 0.1                            | 0.5                           | 0.5  | 123                                         | 19                | -2.2                       | -2.4              |
| 3.0                            | 1.0                            | 0.5                           | 0.5  | 129                                         | 21                | -2.1                       | -2.3              |
| 3.0                            | 3.0                            | 0.5                           | 0.5  | 141                                         | 20                | -2.5                       | -2.7              |
| 3.0                            | 10.0                           | 0.5                           | 0.5  | 156                                         | 18                | -4.7                       | -4.9              |
| 3.0                            | 3.0                            | 0.01                          | 0.5  | 117                                         | 24                | -2.6                       | -2.9              |
| 3.0                            | 3.0                            | 0.1                           | 0.5  | 123                                         | 22                | -2.5                       | -2.6              |
| 3.0                            | 3.0                            | 1.0                           | 0.5  | 123                                         | 25                | -2.3                       | -2.4              |
| 3.0                            | 3.0                            | 5.0                           | 0.5  | 140                                         | 26                | -2.4                       | -2.7              |
| 3.0                            | 3.0                            | 0.5                           | 0.01 | 137                                         | 24                | -2.8                       | -2.9              |
| 3.0                            | 3.0                            | 0.5                           | 0.1  | 124                                         | 22                | -2.5                       | -2.4              |
| 3.0                            | 3.0                            | 0.5                           | 1.0  | 122                                         | 22                | -2.6                       | -2.4              |
| 3.0                            | 3.0                            | 0.5                           | 5.0  | 104                                         | 24                | -2.5                       | -2.6              |

Table 3

| Additives (mole %)             |                                |                               |     |                   | Electrical Properties of Resultant Resistor |                   | Change Rate after DC Life Test (%) |                   | Change Rate after Impulse Test (%) |                   |       |
|--------------------------------|--------------------------------|-------------------------------|-----|-------------------|---------------------------------------------|-------------------|------------------------------------|-------------------|------------------------------------|-------------------|-------|
| Bi <sub>2</sub> O <sub>3</sub> | Co <sub>2</sub> O <sub>3</sub> | B <sub>2</sub> O <sub>3</sub> | MnO | Further additives | <sup>c</sup><br>at a given current of 1 mA  | <sup>c</sup><br>n | <sup>c</sup><br>at 0.005 mA        | <sup>c</sup><br>n | <sup>c</sup><br>n                  | <sup>c</sup><br>n |       |
| 0.1                            | 0.1                            | 0.1                           | 0.1 | MgO               | 0.01                                        | 92                | 28                                 | -2.0              | -2.2                               | -8.8              | -12.5 |
| 0.1                            | 0.1                            | 0.1                           | 0.5 | MgO               | 0.01                                        | 106               | 31                                 | -1.8              | -2.2                               | -8.5              | -11.6 |
| 0.1                            | 0.1                            | 0.1                           | 3.0 | MgO               | 0.01                                        | 122               | 35                                 | -1.9              | -2.0                               | -8.1              | -11.5 |
| 0.5                            | 0.5                            | 1.0                           | 0.1 | MgO               | 1.0                                         | 66                | 27                                 | -2.0              | -2.4                               | -8.8              | -12.7 |
| 0.5                            | 0.5                            | 1.0                           | 0.5 | MgO               | 1.0                                         | 92                | 29                                 | -1.8              | -2.2                               | -8.4              | -11.7 |
| 0.5                            | 0.5                            | 1.0                           | 3.0 | MgO               | 1.0                                         | 113               | 34                                 | -1.6              | -2.5                               | -8.7              | -11.1 |
| 3.0                            | 3.0                            | 5.0                           | 0.1 | MgO               | 5.0                                         | 77                | 26                                 | -1.8              | -2.4                               | -8.6              | -11.3 |
| 3.0                            | 3.0                            | 5.0                           | 0.5 | MgO               | 5.0                                         | 103               | 32                                 | -1.5              | -2.3                               | -8.0              | -11.6 |
| 3.0                            | 3.0                            | 5.0                           | 3.0 | MgO               | 5.0                                         | 137               | 36                                 | -1.6              | -2.1                               | -8.9              | -11.1 |
| 0.1                            | 0.1                            | 0.1                           | 0.1 | CaO               | 0.01                                        | 91                | 29                                 | -1.9              | -2.3                               | -8.8              | -12.7 |
| 0.1                            | 0.1                            | 0.1                           | 0.5 | CaO               | 0.01                                        | 107               | 30                                 | -1.7              | -2.1                               | -8.7              | -11.6 |
| 0.1                            | 0.1                            | 0.1                           | 3.0 | CaO               | 0.01                                        | 121               | 36                                 | -1.8              | -2.1                               | -8.1              | -11.5 |
| 0.5                            | 0.5                            | 1.0                           | 0.1 | CaO               | 1.0                                         | 67                | 26                                 | -1.9              | -2.3                               | -9.0              | -12.7 |
| 0.5                            | 0.5                            | 1.0                           | 0.5 | CaO               | 1.0                                         | 91                | 30                                 | -1.7              | -2.3                               | -8.4              | -11.9 |
| 0.5                            | 0.5                            | 1.0                           | 3.0 | CaO               | 1.0                                         | 114               | 33                                 | -1.5              | -2.4                               | -8.9              | -11.4 |
| 3.0                            | 3.0                            | 5.0                           | 0.1 | CaO               | 5.0                                         | 76                | 27                                 | -1.7              | -2.5                               | -8.6              | -11.5 |
| 3.0                            | 3.0                            | 5.0                           | 0.5 | CaO               | 5.0                                         | 104               | 31                                 | -1.4              | -2.2                               | -8.2              | -15.6 |
| 3.0                            | 3.0                            | 5.0                           | 3.0 | CaO               | 5.0                                         | 136               | 37                                 | -1.5              | -2.2                               | -8.9              | -11.3 |

Table 3 - Continued

| Additives (mole %)             |                                |                               |     |                   | Electrical Properties of Resultant Resistor |     | Change Rate after DC Life Test (%) |      | Change Rate after Impulse Test (%) |       |       |
|--------------------------------|--------------------------------|-------------------------------|-----|-------------------|---------------------------------------------|-----|------------------------------------|------|------------------------------------|-------|-------|
| Bi <sub>2</sub> O <sub>3</sub> | Co <sub>2</sub> O <sub>3</sub> | B <sub>2</sub> O <sub>3</sub> | MnO | Further additives | c at a given current of 1 mA                | n   | c at 0.005 mA                      | n    | c                                  | n     |       |
| 0.1                            | 0.1                            | 0.1                           | 0.1 | BaO               | 0.01                                        | 90  | 27                                 | -2.1 | -2.5                               | -10.2 | -14.9 |
| 0.1                            | 0.1                            | 0.1                           | 0.5 | BaO               | 0.01                                        | 105 | 29                                 | -2.0 | -2.4                               | -9.0  | -14.0 |
| 0.1                            | 0.1                            | 0.1                           | 3.0 | BaO               | 0.01                                        | 120 | 34                                 | -2.0 | -2.3                               | -8.5  | -13.8 |
| 0.5                            | 0.5                            | 1.0                           | 0.1 | BaO               | 1.0                                         | 65  | 25                                 | -2.2 | -2.6                               | -10.3 | -15.1 |
| 0.5                            | 0.5                            | 1.0                           | 0.5 | BaO               | 1.0                                         | 90  | 28                                 | -1.9 | -2.5                               | -9.8  | -14.2 |
| 0.5                            | 0.5                            | 1.0                           | 3.0 | BaO               | 1.0                                         | 112 | 32                                 | -1.8 | -2.7                               | -9.2  | -13.5 |
| 3.0                            | 3.0                            | 5.0                           | 0.1 | BaO               | 5.0                                         | 75  | 25                                 | -1.9 | -2.7                               | -10.0 | -14.8 |
| 3.0                            | 3.0                            | 5.0                           | 0.5 | BaO               | 5.0                                         | 102 | 30                                 | -1.7 | -2.5                               | -9.5  | -14.0 |
| 3.0                            | 3.0                            | 5.0                           | 3.0 | BaO               | 5.0                                         | 135 | 35                                 | -1.7 | -2.4                               | -9.3  | -13.6 |
| 0.1                            | 0.1                            | 0.1                           | 0.1 | SrO               | 0.01                                        | 90  | 27                                 | -1.8 | -2.4                               | -9.7  | -14.3 |
| 0.1                            | 0.1                            | 0.1                           | 0.5 | SrO               | 0.01                                        | 106 | 30                                 | -1.8 | -2.2                               | -8.4  | -13.2 |
| 0.1                            | 0.1                            | 0.1                           | 3.0 | SrO               | 0.01                                        | 120 | 34                                 | -1.7 | -2.2                               | -8.0  | -13.1 |
| 0.5                            | 0.5                            | 1.0                           | 0.1 | SrO               | 1.0                                         | 66  | 26                                 | -2.0 | -2.4                               | -9.7  | -14.3 |
| 0.5                            | 0.5                            | 1.0                           | 0.5 | SrO               | 1.0                                         | 90  | 28                                 | -1.6 | -2.4                               | -9.3  | -13.5 |
| 0.5                            | 0.5                            | 1.0                           | 3.0 | SrO               | 1.0                                         | 113 | 33                                 | -1.6 | -2.5                               | -8.6  | -12.7 |
| 3.0                            | 3.0                            | 5.0                           | 0.1 | SrO               | 5.0                                         | 75  | 25                                 | -1.6 | -2.6                               | -9.5  | -14.1 |
| 3.0                            | 3.0                            | 5.0                           | 0.5 | SrO               | 5.0                                         | 103 | 31                                 | -1.5 | -2.3                               | -8.9  | -13.2 |
| 3.0                            | 3.0                            | 5.0                           | 3.0 | SrO               | 5.0                                         | 135 | 35                                 | -1.4 | -2.3                               | -8.8  | -12.9 |

Table 4

| Additives (mole %)             |                                |                               |     |                                |                  |                   | Electrical Properties of Resultant Resistor |     | Change Rate after DC Life Test (%) |      | Change Rate after Impulse Test (%) |      |      |
|--------------------------------|--------------------------------|-------------------------------|-----|--------------------------------|------------------|-------------------|---------------------------------------------|-----|------------------------------------|------|------------------------------------|------|------|
| Bi <sub>2</sub> O <sub>3</sub> | Co <sub>2</sub> O <sub>3</sub> | B <sub>2</sub> O <sub>3</sub> | MnO | Sb <sub>2</sub> O <sub>3</sub> | TiO <sub>2</sub> | Further Additives | c at 1mA                                    | n   | c at 0.002mA                       | n    | c                                  | n    |      |
| 0.1                            | 0.1                            | 0.1                           | 0.1 | 0.05                           | —                | MgO               | 0.01                                        | 50  | 50                                 | -1.8 | -1.9                               | -6.3 | -7.2 |
| 0.1                            | 0.1                            | 0.1                           | 0.1 | 1.0                            | —                | MgO               | 0.01                                        | 56  | 52                                 | -1.6 | -2.2                               | -6.9 | -7.1 |
| 0.1                            | 0.1                            | 0.1                           | 0.1 | 3.0                            | —                | MgO               | 0.01                                        | 82  | 53                                 | -1.7 | -1.8                               | -6.1 | -7.1 |
| 0.5                            | 0.5                            | 1.0                           | 0.5 | 0.05                           | —                | MgO               | 1.0                                         | 51  | 52                                 | -1.8 | -2.0                               | -6.9 | -7.8 |
| 0.5                            | 0.5                            | 1.0                           | 0.5 | 1.0                            | —                | MgO               | 1.0                                         | 67  | 53                                 | -1.8 | -1.9                               | -6.2 | -7.1 |
| 0.5                            | 0.5                            | 1.0                           | 0.5 | 3.0                            | —                | MgO               | 1.0                                         | 86  | 56                                 | -1.8 | -1.8                               | -6.9 | -7.9 |
| 3.0                            | 3.0                            | 5.0                           | 3.0 | 0.05                           | —                | MgO               | 3.0                                         | 72  | 50                                 | -2.0 | -1.8                               | -6.3 | -7.3 |
| 3.0                            | 3.0                            | 5.0                           | 3.0 | 1.0                            | —                | MgO               | 3.0                                         | 88  | 53                                 | -1.5 | -2.3                               | -6.9 | -7.4 |
| 3.0                            | 3.0                            | 5.0                           | 3.0 | 3.0                            | —                | MgO               | 3.0                                         | 109 | 54                                 | -1.8 | -1.8                               | -6.9 | -7.2 |
| 0.1                            | 0.1                            | 0.1                           | 0.1 | 0.05                           | —                | CaO               | 0.01                                        | 49  | 51                                 | -1.7 | -2.0                               | -6.2 | -7.1 |
| 0.1                            | 0.1                            | 0.1                           | 0.1 | 1.0                            | —                | CaO               | 0.01                                        | 57  | 51                                 | -1.5 | -2.1                               | -6.0 | -7.2 |
| 0.1                            | 0.1                            | 0.1                           | 0.1 | 3.0                            | —                | CaO               | 0.01                                        | 81  | 54                                 | -1.6 | -1.9                               | -6.0 | -7.9 |
| 0.5                            | 0.5                            | 1.0                           | 0.5 | 0.05                           | —                | CaO               | 1.0                                         | 52  | 51                                 | -1.7 | -1.9                               | -6.0 | -7.9 |
| 0.5                            | 0.5                            | 1.0                           | 0.5 | 1.0                            | —                | CaO               | 1.0                                         | 66  | 54                                 | -1.7 | -2.0                               | -6.1 | -7.1 |
| 0.5                            | 0.5                            | 1.0                           | 0.5 | 3.0                            | —                | CaO               | 1.0                                         | 87  | 55                                 | -1.7 | -1.7                               | -6.0 | -7.2 |
| 3.0                            | 3.0                            | 3.0                           | 3.0 | 0.05                           | —                | CaO               | 3.0                                         | 71  | 51                                 | -1.9 | -1.9                               | -6.1 | -7.2 |
| 3.0                            | 3.0                            | 3.0                           | 3.0 | 1.0                            | —                | CaO               | 3.0                                         | 89  | 52                                 | -1.4 | -2.2                               | -6.0 | -7.5 |
| 3.0                            | 3.0                            | 3.0                           | 3.0 | 3.5                            | —                | CaO               | 3.0                                         | 108 | 55                                 | -1.7 | -1.9                               | -6.8 | -7.1 |
| 0.1                            | 0.1                            | 0.1                           | 0.1 | 0.05                           | —                | BaO               | 0.01                                        | 48  | 49                                 | -1.9 | -2.2                               | -6.3 | -7.2 |
| 0.1                            | 0.1                            | 0.1                           | 0.1 | 1.0                            | —                | BaO               | 0.01                                        | 55  | 50                                 | -1.8 | -2.4                               | -6.0 | -7.2 |
| 0.1                            | 0.1                            | 0.1                           | 0.1 | 3.0                            | —                | BaO               | 0.01                                        | 80  | 52                                 | -1.8 | -2.1                               | -6.1 | -7.1 |
| 0.5                            | 0.5                            | 1.0                           | 0.5 | 0.05                           | —                | BaO               | 1.0                                         | 50  | 50                                 | -2.0 | -2.2                               | -7.0 | -7.9 |
| 0.5                            | 0.5                            | 1.0                           | 0.5 | 1.0                            | —                | BaO               | 1.0                                         | 65  | 52                                 | -1.9 | -2.2                               | -7.2 | -7.1 |
| 0.5                            | 0.5                            | 1.0                           | 0.5 | 3.0                            | —                | BaO               | 1.0                                         | 85  | 54                                 | -2.0 | -2.0                               | -7.0 | -7.2 |
| 3.0                            | 3.0                            | 3.0                           | 3.0 | 0.05                           | —                | BaO               | 3.0                                         | 70  | 49                                 | -2.1 | -2.1                               | -7.3 | -7.3 |
| 3.0                            | 3.0                            | 3.0                           | 3.0 | 1.0                            | —                | BaO               | 3.0                                         | 87  | 51                                 | -1.7 | -2.5                               | -7.0 | -7.5 |
| 3.0                            | 3.0                            | 3.0                           | 3.0 | 3.0                            | —                | BaO               | 3.0                                         | 107 | 53                                 | -1.9 | -2.1                               | -7.9 | -7.2 |
| 0.1                            | 0.1                            | 0.1                           | 0.1 | 0.05                           | —                | SrO               | 0.01                                        | 48  | 49                                 | -1.6 | -2.1                               | -7.2 | -7.1 |
| 0.1                            | 0.1                            | 0.1                           | 0.1 | 1.0                            | —                | SrO               | 0.01                                        | 56  | 51                                 | -1.6 | -2.2                               | -7.8 | -7.2 |
| 0.1                            | 0.1                            | 0.1                           | 0.1 | 3.0                            | —                | SrO               | 0.01                                        | 80  | 52                                 | -1.5 | -2.0                               | -7.0 | -7.9 |
| 0.5                            | 0.5                            | 1.0                           | 0.5 | 0.05                           | —                | SrO               | 1.0                                         | 51  | 51                                 | -1.8 | -2.0                               | -7.8 | -7.7 |
| 0.5                            | 0.5                            | 1.0                           | 0.5 | 1.0                            | —                | SrO               | 1.0                                         | 65  | 52                                 | -1.6 | -2.1                               | -7.1 | -7.2 |
| 0.5                            | 0.5                            | 1.0                           | 0.5 | 3.0                            | —                | SrO               | 1.0                                         | 86  | 55                                 | -1.8 | -1.8                               | -7.8 | -7.8 |
| 3.0                            | 3.0                            | 3.0                           | 3.0 | 0.05                           | —                | SrO               | 3.0                                         | 70  | 49                                 | -1.8 | -2.0                               | -7.2 | -7.2 |
| 3.0                            | 3.0                            | 3.0                           | 3.0 | 1.0                            | —                | SrO               | 3.0                                         | 88  | 52                                 | -1.5 | -2.3                               | -7.8 | -7.3 |
| 3.0                            | 3.0                            | 3.0                           | 3.0 | 3.0                            | —                | SrO               | 3.0                                         | 107 | 53                                 | -1.6 | -2.0                               | -7.8 | -7.1 |
| 0.1                            | 0.1                            | 0.1                           | 0.1 | —                              | 0.1              | MgO               | 0.01                                        | 22  | 31                                 | -2.2 | -1.9                               | -7.4 | -8.7 |
| 0.1                            | 0.1                            | 0.1                           | 0.1 | —                              | 1.0              | MgO               | 0.01                                        | 8   | 32                                 | -1.8 | -2.0                               | -6.8 | -8.3 |
| 0.1                            | 0.1                            | 0.1                           | 0.1 | —                              | 3.0              | MgO               | 0.01                                        | 7   | 30                                 | -1.8 | -2.1                               | -6.9 | -8.4 |
| 0.5                            | 0.5                            | 1.0                           | 0.5 | —                              | 0.1              | MgO               | 1.0                                         | 26  | 32                                 | -1.8 | -1.9                               | -6.8 | -9.3 |
| 0.5                            | 0.5                            | 1.0                           | 0.5 | —                              | 1.0              | MgO               | 1.0                                         | 10  | 32                                 | -1.6 | -1.8                               | 6.7  | 8.4  |
| 0.5                            | 0.5                            | 1.0                           | 0.5 | —                              | 3.0              | MgO               | 1.0                                         | 8   | 32                                 | -1.6 | -2.0                               | 6.3  | 8.6  |
| 3.0                            | 3.0                            | 3.0                           | 3.0 | —                              | 0.1              | MgO               | 3.0                                         | 50  | 32                                 | -2.0 | -1.7                               | 6.6  | 9.0  |
| 3.0                            | 3.0                            | 3.0                           | 3.0 | —                              | 1.0              | MgO               | 3.0                                         | 31  | 32                                 | -1.6 | -1.8                               | 6.3  | 8.6  |
| 3.0                            | 3.0                            | 3.0                           | 3.0 | —                              | 3.0              | MgO               | 3.0                                         | 29  | 31                                 | -1.8 | -2.0                               | 5.9  | 8.8  |

Table 4—Continued

| Additives (mole %)             |                                |                               |     |                                |                  |                   | Electrical Properties of Resultant Resistor |    | Change Rate after DC Life Test (%) |      | Change Rate after Impulse Test (%) |       |
|--------------------------------|--------------------------------|-------------------------------|-----|--------------------------------|------------------|-------------------|---------------------------------------------|----|------------------------------------|------|------------------------------------|-------|
| Bi <sub>2</sub> O <sub>3</sub> | Co <sub>2</sub> O <sub>3</sub> | B <sub>2</sub> O <sub>3</sub> | MnO | Sb <sub>2</sub> O <sub>3</sub> | TiO <sub>2</sub> | Further Additives | c at 1mA                                    | n  | c at 0.002mA                       | n    | c                                  | n     |
| 0.1                            | 0.1                            | 0.1                           | 0.1 | —                              | 0.1              | CaO 0.01          | 21                                          | 32 | -2.1                               | -2.0 | -7.3                               | -8.8  |
| 0.1                            | 0.1                            | 0.1                           | 0.1 | —                              | 1.0              | CaO 0.01          | 9                                           | 31 | -1.7                               | -1.9 | -6.7                               | -8.2  |
| 0.1                            | 0.1                            | 0.1                           | 0.1 | —                              | 3.0              | CaO 0.01          | 6                                           | 31 | -1.7                               | -2.2 | -6.8                               | -8.5  |
| 0.5                            | 0.5                            | 1.0                           | 0.5 | —                              | 0.1              | CaO 1.0           | 27                                          | 32 | -1.7                               | -1.8 | -6.7                               | -8.4  |
| 0.5                            | 0.5                            | 1.0                           | 0.5 | —                              | 1.0              | CaO 1.0           | 9                                           | 32 | -1.5                               | -1.9 | -6.6                               | -8.6  |
| 0.5                            | 0.5                            | 1.0                           | 0.5 | —                              | 3.0              | CaO 1.0           | 9                                           | 31 | -1.5                               | -1.9 | -6.2                               | -8.5  |
| 3.0                            | 3.0                            | 3.0                           | 3.0 | —                              | 0.1              | CaO 3.0           | 49                                          | 33 | -1.9                               | -1.8 | -6.5                               | -9.1  |
| 3.0                            | 3.0                            | 3.0                           | 3.0 | —                              | 1.0              | CaO 3.0           | 32                                          | 31 | -1.5                               | -1.7 | -6.2                               | -8.5  |
| 3.0                            | 3.0                            | 3.0                           | 3.0 | —                              | 3.0              | CaO 3.0           | 28                                          | 32 | -1.7                               | -2.1 | -5.8                               | -8.9  |
| 0.1                            | 0.1                            | 0.1                           | 0.1 | —                              | 0.1              | BaO 0.01          | 20                                          | 30 | -2.3                               | -2.2 | -7.5                               | -11.0 |
| 0.1                            | 0.1                            | 0.1                           | 0.1 | —                              | 1.0              | BaO 0.01          | 7                                           | 30 | -2.0                               | -2.2 | -7.0                               | -10.5 |
| 0.1                            | 0.1                            | 0.1                           | 0.1 | —                              | 3.0              | BaO 0.01          | 5                                           | 29 | -1.9                               | -2.4 | -7.0                               | -10.7 |
| 0.5                            | 0.5                            | 1.0                           | 0.5 | —                              | 0.1              | BaO 1.0           | 25                                          | 30 | -2.0                               | -2.1 | -7.0                               | -11.0 |
| 0.5                            | 0.5                            | 1.0                           | 0.5 | —                              | 1.0              | BaO 1.0           | 8                                           | 31 | -1.7                               | -2.1 | -6.8                               | -10.7 |
| 0.5                            | 0.5                            | 1.0                           | 0.5 | —                              | 3.0              | BaO 1.0           | 7                                           | 30 | -1.8                               | -2.2 | -6.5                               | -10.8 |
| 3.0                            | 3.0                            | 3.0                           | 3.0 | —                              | 0.1              | BaO 3.0           | 48                                          | 31 | -2.1                               | -2.0 | -6.7                               | -11.3 |
| 3.0                            | 3.0                            | 3.0                           | 3.0 | —                              | 1.0              | BaO 3.0           | 30                                          | 30 | -1.8                               | -2.0 | -6.5                               | -10.8 |
| 3.0                            | 3.0                            | 3.0                           | 3.0 | —                              | 3.0              | BaO 3.0           | 27                                          | 30 | -1.9                               | -2.3 | -6.0                               | -11.1 |
| 0.1                            | 0.1                            | 0.1                           | 0.1 | —                              | 0.1              | SrO 0.01          | 20                                          | 30 | -2.0                               | -2.1 | -7.2                               | -10.9 |
| 0.1                            | 0.1                            | 0.1                           | 0.1 | —                              | 1.0              | SrO 0.01          | 8                                           | 31 | -1.8                               | -2.0 | -6.8                               | -10.3 |
| 0.1                            | 0.1                            | 0.1                           | 0.1 | —                              | 3.0              | SrO 0.01          | 5                                           | 29 | -1.6                               | -2.3 | -6.7                               | -10.6 |
| 0.5                            | 0.5                            | 1.0                           | 0.5 | —                              | 0.1              | SrO 1.0           | 26                                          | 31 | -1.8                               | -1.9 | -6.8                               | -11.0 |
| 0.5                            | 0.5                            | 1.0                           | 0.5 | —                              | 1.0              | SrO 1.0           | 8                                           | 30 | -1.4                               | -2.0 | -6.5                               | -10.6 |
| 0.5                            | 0.5                            | 1.0                           | 0.5 | —                              | 3.0              | SrO 1.0           | 8                                           | 31 | -1.6                               | -2.0 | -6.3                               | -10.6 |
| 3.0                            | 3.0                            | 3.0                           | 3.0 | —                              | 0.1              | SrO 3.0           | 48                                          | 32 | -1.9                               | -1.9 | -6.4                               | -11.0 |
| 3.0                            | 3.0                            | 3.0                           | 3.0 | —                              | 1.0              | SrO 3.0           | 31                                          | 31 | -1.6                               | -1.8 | -6.3                               | -10.6 |
| 3.0                            | 3.0                            | 3.0                           | 3.0 | —                              | 3.0              | SrO 3.0           | 27                                          | 30 | -1.6                               | -2.2 | -5.8                               | -11.0 |

TABLE 5

| Additives (mole percent)       |                                |     |                  |                               |     |                                | Electrical properties of resultant resistor |          | Change rate after DC life test (percent) |                 | Change rate after impulse test (percent) |      |      |
|--------------------------------|--------------------------------|-----|------------------|-------------------------------|-----|--------------------------------|---------------------------------------------|----------|------------------------------------------|-----------------|------------------------------------------|------|------|
| Bi <sub>2</sub> O <sub>3</sub> | Co <sub>2</sub> O <sub>3</sub> | MnO | TiO <sub>2</sub> | B <sub>2</sub> O <sub>3</sub> | NiO | Cr <sub>2</sub> O <sub>3</sub> | Further additives                           | At 1 ma. | n                                        | Δc at 0.001 ma. | Δn                                       | Δc   | Δn   |
| 0.1                            | 0.1                            | 0.1 | 0.1              | 0.1                           | 0.1 | 0.1                            | MgO 0.01                                    | 9        | 29                                       | -2.4            | -1.7                                     | -3.6 | -5.2 |
| 0.1                            | 0.1                            | 0.1 | 0.1              | 0.1                           | 0.5 | 0.5                            | MgO 0.01                                    | 15       | 31                                       | -2.0            | -1.8                                     | -3.3 | -5.1 |
| 0.1                            | 0.1                            | 0.1 | 0.1              | 0.1                           | 3.0 | 3.0                            | MgO 0.01                                    | 30       | 32                                       | -1.9            | -1.9                                     | -3.2 | -5.8 |
| 0.5                            | 0.5                            | 0.5 | 1.0              | 1.0                           | 0.1 | 0.1                            | MgO 1.0                                     | 12       | 31                                       | -2.2            | -1.7                                     | -3.4 | -5.2 |
| 0.5                            | 0.5                            | 0.5 | 1.0              | 1.0                           | 0.5 | 0.5                            | MgO 1.0                                     | 19       | 33                                       | -2.0            | -1.6                                     | -3.2 | -4.9 |
| 0.5                            | 0.5                            | 0.5 | 1.0              | 1.0                           | 3.0 | 3.0                            | MgO 1.0                                     | 32       | 32                                       | -1.8            | -1.8                                     | -3.8 | -5.3 |
| 3.0                            | 3.0                            | 3.0 | 3.0              | 3.0                           | 0.1 | 0.1                            | MgO 3.0                                     | 27       | 31                                       | -2.2            | -1.6                                     | -3.7 | -5.7 |
| 3.0                            | 3.0                            | 3.0 | 3.0              | 3.0                           | 0.5 | 0.5                            | MgO 3.0                                     | 33       | 33                                       | -2.0            | -1.7                                     | -3.5 | -5.8 |
| 3.0                            | 3.0                            | 3.0 | 3.0              | 3.0                           | 3.0 | 3.0                            | MgO 3.0                                     | 42       | 34                                       | -2.0            | -1.9                                     | -2.9 | -4.4 |
| 0.1                            | 0.1                            | 0.1 | 0.1              | 0.1                           | 0.1 | 0.1                            | CaO 0.01                                    | 8        | 30                                       | -2.3            | -1.8                                     | -3.5 | -5.3 |
| 0.1                            | 0.1                            | 0.1 | 0.1              | 0.1                           | 0.5 | 0.5                            | CaO 0.01                                    | 16       | 30                                       | -1.8            | -1.7                                     | -3.2 | -5.0 |
| 0.1                            | 0.1                            | 0.1 | 0.1              | 0.1                           | 3.0 | 3.0                            | CaO 0.01                                    | 29       | 33                                       | -1.8            | -2.0                                     | -3.1 | -4.9 |
| 0.5                            | 0.5                            | 0.5 | 1.0              | 1.0                           | 0.1 | 0.1                            | CaO 1.0                                     | 13       | 30                                       | -2.1            | -1.6                                     | -3.3 | -5.1 |
| 0.5                            | 0.5                            | 0.5 | 1.0              | 1.0                           | 0.5 | 0.5                            | CaO 1.0                                     | 18       | 33                                       | -1.9            | -1.7                                     | -3.1 | -5.0 |
| 0.5                            | 0.5                            | 0.5 | 1.0              | 1.0                           | 3.0 | 3.0                            | CaO 1.0                                     | 33       | 31                                       | -1.7            | -1.7                                     | -3.7 | -6.7 |
| 3.0                            | 3.0                            | 3.0 | 3.0              | 3.0                           | 0.1 | 0.1                            | CaO 3.0                                     | 26       | 32                                       | -2.1            | -1.7                                     | -3.6 | -6.5 |
| 3.0                            | 3.0                            | 3.0 | 3.0              | 3.0                           | 0.5 | 0.5                            | CaO 3.0                                     | 34       | 32                                       | -1.9            | -1.6                                     | -3.4 | -5.2 |
| 3.0                            | 3.0                            | 3.0 | 3.0              | 3.0                           | 3.0 | 3.0                            | CaO 3.0                                     | 41       | 35                                       | -1.9            | -1.9                                     | -2.8 | -4.8 |
| 0.1                            | 0.1                            | 0.1 | 0.1              | 0.1                           | 0.1 | 0.1                            | CaO 0.01                                    | 7        | 28                                       | -2.5            | -2.0                                     | -4.7 | -6.5 |
| 0.1                            | 0.1                            | 0.1 | 0.1              | 0.1                           | 0.5 | 0.5                            | CaO 0.01                                    | 14       | 29                                       | -2.2            | -2.0                                     | -4.5 | -6.3 |
| 0.1                            | 0.1                            | 0.1 | 0.1              | 0.1                           | 3.0 | 3.0                            | CaO 0.01                                    | 28       | 31                                       | -2.0            | -2.2                                     | -4.3 | -6.1 |
| 0.5                            | 0.5                            | 0.5 | 1.0              | 1.0                           | 0.1 | 0.1                            | BaO 1.0                                     | 11       | 29                                       | -2.4            | -1.9                                     | -4.6 | -6.4 |
| 0.5                            | 0.5                            | 0.5 | 1.0              | 1.0                           | 0.5 | 0.5                            | BaO 1.0                                     | 17       | 32                                       | -2.1            | -1.9                                     | -4.3 | -6.2 |
| 0.5                            | 0.5                            | 0.5 | 1.0              | 1.0                           | 3.0 | 3.0                            | BaO 1.0                                     | 31       | 30                                       | -2.0            | -2.0                                     | -5.0 | -7.0 |
| 3.0                            | 3.0                            | 3.0 | 3.0              | 3.0                           | 0.1 | 0.1                            | BaO 3.0                                     | 25       | 30                                       | -2.3            | -1.9                                     | -4.8 | -6.7 |
| 3.0                            | 3.0                            | 3.0 | 3.0              | 3.0                           | 0.5 | 0.5                            | BaO 3.0                                     | 32       | 31                                       | -2.2            | -1.9                                     | -4.7 | -6.5 |
| 3.0                            | 3.0                            | 3.0 | 3.0              | 3.0                           | 3.0 | 3.0                            | BaO 3.0                                     | 40       | 33                                       | -2.1            | -2.1                                     | -4.0 | -6.0 |
| 0.1                            | 0.1                            | 0.1 | 0.1              | 0.1                           | 0.1 | 0.1                            | SrO 0.01                                    | 7        | 28                                       | -2.2            | -1.9                                     | -4.4 | -6.4 |
| 0.1                            | 0.1                            | 0.1 | 0.1              | 0.1                           | 0.5 | 0.5                            | SrO 0.01                                    | 15       | 30                                       | -2.0            | -1.8                                     | -4.3 | -6.1 |
| 0.1                            | 0.1                            | 0.1 | 0.1              | 0.1                           | 3.0 | 3.0                            | SrO 0.01                                    | 28       | 31                                       | -1.7            | -2.1                                     | -4.0 | -6.0 |
| 0.5                            | 0.5                            | 0.5 | 1.0              | 1.0                           | 0.1 | 0.1                            | SrO 1.0                                     | 12       | 30                                       | -2.2            | -1.7                                     | -4.4 | -6.2 |
| 0.5                            | 0.5                            | 0.5 | 1.0              | 1.0                           | 0.5 | 0.5                            | SrO 1.0                                     | 17       | 32                                       | -1.8            | -1.8                                     | -4.0 | -6.1 |
| 0.5                            | 0.5                            | 0.5 | 1.0              | 1.0                           | 3.0 | 3.0                            | SrO 1.0                                     | 32       | 31                                       | -1.8            | -1.8                                     | -4.8 | -6.8 |
| 3.0                            | 3.0                            | 3.0 | 3.0              | 3.0                           | 0.1 | 0.1                            | SrO 3.0                                     | 25       | 30                                       | -2.0            | -1.9                                     | -4.5 | -6.6 |
| 3.1                            | 3.0                            | 3.0 | 3.0              | 3.0                           | 0.5 | 0.5                            | SrO 3.0                                     | 33       | 32                                       | -2.0            | -1.7                                     | -4.5 | -6.3 |
| 3.1                            | 3.0                            | 3.0 | 3.0              | 3.0                           | 3.0 | 3.0                            | SrO 3.0                                     | 40       | 33                                       | -1.8            | -1.9                                     | -3.7 | -5.9 |
| 0.1                            | 0.1                            | 0.1 | 0.1              | 0.1                           | 0.1 | 0.1                            | 0.01 MgO                                    | 9        | 30                                       | -2.7            | -2.0                                     | -4.2 | -4.2 |
| 0.1                            | 0.1                            | 0.1 | 0.1              | 0.1                           | 0.5 | 0.5                            | 0.01 MgO                                    | 10       | 31                                       | -2.4            | -2.1                                     | -4.2 | -4.2 |
| 0.1                            | 0.1                            | 0.1 | 0.1              | 0.1                           | 3.0 | 3.0                            | 0.01 MgO                                    | 22       | 31                                       | -2.4            | -1.9                                     | -4.3 | -4.0 |
| 0.5                            | 0.5                            | 0.5 | 1.0              | 1.0                           | 0.1 | 0.1                            | 0.01 MgO                                    | 11       | 31                                       | -2.4            | -1.9                                     | -4.3 | -4.2 |
| 0.5                            | 0.5                            | 0.5 | 1.0              | 1.0                           | 0.5 | 0.5                            | 0.01 MgO                                    | 14       | 31                                       | -2.7            | -1.8                                     | -2.2 | -3.9 |

TABLE 5—Continued

| Additives (mole percent)       |                                |     |                  |                               |     |                                |                   | Electrical properties of resultant resistor |    | Change rate after DC life test (percent) |      | Change rate after impulse test (percent) |      |      |
|--------------------------------|--------------------------------|-----|------------------|-------------------------------|-----|--------------------------------|-------------------|---------------------------------------------|----|------------------------------------------|------|------------------------------------------|------|------|
| Bi <sub>2</sub> O <sub>3</sub> | Co <sub>2</sub> O <sub>3</sub> | MnO | TiO <sub>2</sub> | B <sub>2</sub> O <sub>3</sub> | NiO | Cr <sub>2</sub> O <sub>3</sub> | Further additives | At 1 ma.                                    | n  | Δc at 0.001 ma.                          | Δn   | Δc                                       | Δn   |      |
| 0.5                            | 0.5                            | 0.5 | 1.0              | 1.0                           | —   | 3.0                            | MgO               | 1.0                                         | 26 | -2.5                                     | -2.0 | -2.6                                     | -4.0 |      |
| 3.0                            | 3.0                            | 3.0 | 2.0              | 3.0                           | —   | 0.01                           | MgO               | 3.0                                         | 32 | -2.6                                     | -1.7 | -2.6                                     | -4.4 |      |
| 3.0                            | 3.0                            | 3.0 | 3.0              | 3.0                           | —   | 0.5                            | MgO               | 3.0                                         | 33 | -2.4                                     | -1.8 | -2.5                                     | -4.5 |      |
| 3.0                            | 3.0                            | 3.0 | 3.0              | 3.0                           | —   | 3.0                            | MgO               | 3.0                                         | 49 | -2.4                                     | -1.9 | -2.4                                     | -4.0 |      |
| 0.1                            | 0.1                            | 0.1 | 0.1              | 0.1                           | —   | 0.01                           | CaO               | 0.01                                        | 8  | 31                                       | -2.6 | -2.1                                     | -2.3 | -4.3 |
| 0.1                            | 0.1                            | 0.1 | 0.1              | 0.1                           | —   | 0.5                            | CaO               | 0.01                                        | 11 | 30                                       | -2.3 | -2.0                                     | -2.1 | -4.1 |
| 0.1                            | 0.1                            | 0.1 | 0.1              | 0.1                           | —   | 3.0                            | CaO               | 0.01                                        | 21 | 32                                       | -2.3 | -2.0                                     | -2.2 | -4.1 |
| 0.5                            | 0.5                            | 0.5 | 1.0              | 1.0                           | —   | 0.01                           | CaO               | 1.0                                         | 12 | 30                                       | -2.3 | -1.8                                     | -2.2 | -4.1 |
| 0.5                            | 0.5                            | 0.5 | 1.0              | 1.0                           | —   | 0.5                            | CaO               | 1.0                                         | 13 | 32                                       | -2.6 | -1.9                                     | -2.1 | -4.0 |
| 0.5                            | 0.5                            | 0.5 | 1.0              | 1.0                           | —   | 3.0                            | CaO               | 1.0                                         | 27 | 34                                       | -2.4 | -1.9                                     | -2.5 | -4.9 |
| 3.0                            | 3.0                            | 3.0 | 3.0              | 3.0                           | —   | 0.01                           | CaO               | 3.0                                         | 31 | 32                                       | -2.5 | -1.8                                     | -2.5 | -4.5 |
| 3.0                            | 3.0                            | 3.0 | 3.0              | 3.0                           | —   | 0.5                            | CaO               | 3.0                                         | 34 | 35                                       | -2.3 | -1.7                                     | -2.4 | -4.4 |
| 3.0                            | 3.0                            | 3.0 | 3.0              | 3.0                           | —   | 3.0                            | CaO               | 3.0                                         | 48 | 36                                       | -2.3 | -2.0                                     | -2.3 | -4.1 |
| 0.1                            | 0.1                            | 0.1 | 0.1              | 0.1                           | —   | 0.01                           | BaO               | 0.01                                        | 7  | 29                                       | -2.8 | -2.3                                     | -3.5 | -4.5 |
| 0.1                            | 0.1                            | 1.0 | 0.1              | 0.1                           | —   | 0.5                            | BaO               | 0.01                                        | 9  | 29                                       | -2.6 | -2.3                                     | -3.4 | -4.4 |
| 0.1                            | 0.1                            | 1.0 | 0.1              | 0.1                           | —   | 3.0                            | BaO               | 0.01                                        | 20 | 30                                       | -2.5 | -2.2                                     | -3.4 | -4.3 |
| 0.5                            | 0.5                            | 0.5 | 1.0              | 1.0                           | —   | 0.01                           | BaO               | 1.0                                         | 10 | 29                                       | -2.6 | -2.1                                     | -3.5 | -4.4 |
| 0.5                            | 0.5                            | 0.5 | 1.0              | 1.0                           | —   | 0.5                            | BaO               | 1.0                                         | 12 | 30                                       | -2.8 | -2.1                                     | -3.3 | -4.2 |
| 0.5                            | 0.5                            | 0.5 | 1.0              | 1.0                           | —   | 3.0                            | BaO               | 1.0                                         | 25 | 33                                       | -2.7 | -2.2                                     | -3.8 | -5.7 |
| 3.0                            | 3.0                            | 3.0 | 3.0              | 3.0                           | —   | 0.01                           | BaO               | 3.0                                         | 30 | 30                                       | -2.7 | -2.0                                     | -3.7 | -4.7 |
| 3.0                            | 3.0                            | 3.0 | 3.0              | 3.0                           | —   | 0.5                            | BaO               | 3.0                                         | 32 | 34                                       | -2.6 | -2.0                                     | -3.7 | -4.2 |
| 3.0                            | 3.0                            | 3.0 | 3.0              | 3.0                           | —   | 3.0                            | BaO               | 3.0                                         | 47 | 34                                       | -2.5 | -2.2                                     | -3.5 | -4.3 |
| 0.1                            | 0.1                            | 0.1 | 0.1              | 0.1                           | —   | 0.01                           | SrO               | 0.01                                        | 7  | 29                                       | -2.5 | -2.2                                     | -3.2 | -4.4 |
| 0.1                            | 0.1                            | 0.1 | 0.1              | 0.1                           | —   | 0.5                            | SrO               | 0.01                                        | 10 | 30                                       | -2.4 | -2.1                                     | -3.2 | -4.2 |
| 0.1                            | 0.1                            | 0.1 | 0.1              | 0.1                           | —   | 3.0                            | SrO               | 0.01                                        | 20 | 30                                       | -2.2 | -2.1                                     | -3.1 | -4.2 |
| 0.5                            | 0.5                            | 0.5 | 1.0              | 1.0                           | —   | 0.01                           | SrO               | 1.0                                         | 11 | 30                                       | -2.4 | -1.9                                     | -3.3 | -4.2 |
| 0.5                            | 0.5                            | 0.5 | 1.0              | 1.0                           | —   | 0.5                            | SrO               | 1.0                                         | 12 | 30                                       | -2.5 | -2.0                                     | -3.0 | -4.1 |
| 0.5                            | 0.5                            | 0.5 | 1.0              | 1.0                           | —   | 3.0                            | SrO               | 1.0                                         | 26 | 34                                       | -2.5 | -2.0                                     | -3.6 | -5.0 |
| 3.0                            | 3.0                            | 3.0 | 3.0              | 3.0                           | —   | 0.01                           | SrO               | 3.0                                         | 30 | 30                                       | -2.4 | -1.9                                     | -3.4 | -4.6 |
| 3.0                            | 3.0                            | 3.0 | 3.0              | 3.0                           | —   | 0.5                            | SrO               | 3.0                                         | 33 | 35                                       | -2.4 | -1.8                                     | -3.5 | -4.5 |
| 3.0                            | 3.0                            | 3.0 | 3.0              | 3.0                           | —   | 3.0                            | SrO               | 3.0                                         | 47 | 34                                       | -2.2 | -2.1                                     | -3.2 | -4.2 |
| 0.1                            | 0.1                            | 0.1 | 0.1              | 0.1                           | 0.1 | 0.01                           | MgO               | 0.01                                        | 12 | 35                                       | -1.9 | -2.0                                     | -1.2 | -1.0 |
| 0.1                            | 0.1                            | 0.1 | 0.1              | 0.1                           | 0.1 | 0.5                            | MgO               | 0.01                                        | 18 | 37                                       | -1.8 | -2.0                                     | -1.1 | -1.9 |
| 0.1                            | 0.1                            | 0.1 | 0.1              | 0.1                           | 0.1 | 3.0                            | MgO               | 0.01                                        | 32 | 38                                       | -1.8 | -1.9                                     | -1.0 | -1.9 |
| 0.5                            | 0.5                            | 0.5 | 1.0              | 1.0                           | 0.5 | 0.01                           | MgO               | 1.0                                         | 14 | 34                                       | -1.8 | -1.9                                     | -1.2 | -1.8 |
| 0.5                            | 0.5                            | 0.5 | 1.0              | 1.0                           | 0.5 | 0.5                            | MgO               | 1.0                                         | 19 | 36                                       | -1.7 | -1.9                                     | -0.6 | -0.8 |
| 0.5                            | 0.5                            | 0.5 | 1.0              | 1.0                           | 0.5 | 3.0                            | MgO               | 1.0                                         | 35 | 37                                       | -1.5 | -1.8                                     | -1.1 | -1.7 |
| 3.0                            | 3.0                            | 3.0 | 3.0              | 3.0                           | 3.0 | 3.0                            | MgO               | 3.0                                         | 28 | 36                                       | -1.9 | -1.9                                     | -1.3 | -1.6 |
| 3.0                            | 3.0                            | 3.0 | 3.0              | 3.0                           | 3.0 | 3.0                            | MgO               | 3.0                                         | 35 | 37                                       | -1.8 | -1.8                                     | -1.1 | -1.5 |
| 3.0                            | 3.0                            | 3.0 | 3.0              | 3.0                           | 3.0 | 3.0                            | MgO               | 3.0                                         | 49 | 38                                       | -1.6 | -1.8                                     | -1.0 | -1.5 |
| 0.5                            | 0.5                            | 0.5 | 1.0              | 1.0                           | 0.5 | 0.01                           | CaO               | 1.0                                         | 15 | 34                                       | -1.9 | -2.0                                     | -1.4 | -1.1 |
| 0.5                            | 0.5                            | 0.5 | 1.0              | 1.0                           | 0.5 | 0.5                            | CaO               | 1.0                                         | 20 | 35                                       | -1.9 | -2.1                                     | -1.0 | -0.9 |
| 0.5                            | 0.5                            | 0.5 | 1.0              | 1.0                           | 0.5 | 3.0                            | CaO               | 1.0                                         | 37 | 35                                       | -1.7 | -1.8                                     | -1.2 | -1.3 |
| 0.5                            | 0.5                            | 0.5 | 1.0              | 1.0                           | 0.5 | 0.5                            | BaO               | 1.0                                         | 21 | 36                                       | -1.9 | -2.2                                     | -0.7 | -1.2 |
| 0.5                            | 0.5                            | 0.5 | 1.0              | 1.0                           | 0.5 | 0.5                            | SrO               | 1.0                                         | 23 | 37                                       | -2.1 | -2.3                                     | -0.8 | -0.7 |
| 0.5                            | 0.5                            | 0.5 | 1.0              | 1.0                           | 0.5 | 0.5                            | BaO               | 1.0                                         | 25 | 35                                       | -1.7 | -1.8                                     | -0.7 | -0.9 |
| 0.5                            | 0.5                            | 0.5 | 1.0              | 1.0                           | 0.5 | 0.5                            | CaO               | 1.0                                         | 27 | 37                                       | -1.5 | -1.7                                     | -0.6 | -0.8 |
| 0.5                            | 0.5                            | 0.5 | 1.0              | 1.0                           | 0.5 | 0.5                            | SrO               | 1.0                                         | 25 | 36                                       | -1.4 | -1.5                                     | -0.6 | -0.9 |
| 0.5                            | 0.5                            | 0.5 | 1.0              | 1.0                           | 0.5 | 0.5                            | BaO               | 1.0                                         | 27 | 36                                       | -1.4 | -1.5                                     | -0.5 | -0.9 |
| 0.5                            | 0.5                            | 0.5 | 1.0              | 1.0                           | 0.5 | 0.5                            | BaO               | 1.0                                         | 29 | 37                                       | -1.3 | -1.4                                     | -0.5 | -0.8 |
| 0.5                            | 0.5                            | 0.5 | 1.0              | 1.0                           | 0.5 | 0.5                            | SrO               | 1.0                                         | 30 | 37                                       | -1.2 | -1.4                                     | -0.5 | -0.8 |
| 0.5                            | 0.5                            | 0.5 | 1.0              | 1.0                           | 0.5 | 0.5                            | BaO               | 0.5                                         | 33 | 40                                       | -0.5 | -0.7                                     | -0.5 | -0.6 |

What we claim is:

1. A voltage-nonlinear resistor of the bulk type comprising a sintered body consisting essentially of, as a major part, zinc oxide (ZnO) and, as an additive, 0.01 to 10.0 mole percent of bismuth oxide (Bi<sub>2</sub>O<sub>3</sub>), 0.01 to 10.0 mole percent of cobalt oxide (Co<sub>2</sub>O<sub>3</sub>), 0.01 to 5.0 mole percent of boron trioxide (B<sub>2</sub>O<sub>3</sub>) and 0.01 to 5.0 mole percent of at least one member selected from the group consisting of magnesium oxide (MgO), calcium oxide (CaO), barium oxide (BaO) and strontium oxide (SrO) and electrodes in contact with said body.
2. Voltage-nonlinear resistor according to claim 1, wherein said additive consists essentially of 0.1 to 3.0 mole percent of bismuth oxide (Bi<sub>2</sub>O<sub>3</sub>), 0.1 to 3.0 mole percent of cobalt oxide (Co<sub>2</sub>O<sub>3</sub>), 0.01 to 5.0 mole per-

cent of boron trioxide (B<sub>2</sub>O<sub>3</sub>) and 0.01 to 5.0 mole percent of at least one member selected from the group consisting of magnesium oxide (MgO), calcium oxide (CaO), barium oxide (BaO) and strontium oxide (SrO).

3. Voltage-nonlinear resistor according to claim 2, wherein said sintered body further includes, as an additive, 0.1 to 3.0 mole percent of manganese oxide (MnO).

4. Voltage-nonlinear resistor according to claim 3, wherein said sintered body further includes, as an additive, one member selected from the group consisting of 0.05 to 3.0 mole percent of antimony oxide (Sb<sub>2</sub>O<sub>3</sub>) and 0.1 to 3.0 mole percent of titanium oxide (TiO<sub>2</sub>).

5. Voltage-nonlinear resistor according to claim 3,

wherein said sintered body further includes, as an additive, 0.1 to 3.0 mole percent of titanium oxide ( $TiO_2$ ) and at least one member selected from the group consisting of 0.01 to 3.0 mole percent of chromium oxide

( $Cr_2O_3$ ) and 0.1 to 3.0 mole percent of nickel oxide ( $NiO$ ):

\* \* \* \* \*

5

10

15

20

25

30

35

40

45

50

55

60

65